# EUROPEAN PATENT SPECIFICATION

(11) **EP 2 443 275 B1**
(45) Date of publication and mention of the grant of the patent: **29.06.2016**
(21) Application number: 10723907.1
(22) Date of filing: 03.05.2010
(51) Int. Cl.: D01F 1/10, D01F 2/00

(54) **ULTRAVIOLET PROTECTIVE FABRICS BASED ON MAN-MADE CELLULOSIC FIBRES**
GEGEN ULTRAVIOLETTE STRAHLEN SCHÜTZENDE GEWEBE AUF BASIS VON KUNSTFASERN AUS CELLULOSE
TISSUS PROTÉGEANT CONTRE LES UV À BASE DE FIBRES ARTIFICIELLES DE CELLULOSE

(30) Priority: 15.06.2009 AT 9112009
(43) Date of publication of application: 25.04.2012
(73) Proprietor: Lenzing AG, 4860 Lenzing (AT)
(72) Inventor: BISJAK, Clemens, A-4852 Weyregg (AT); GÜRTLER, Andreas, A-4852 Weyregg (AT); DOBSON, Peter, Derby DE72 3FW (GB); KÄMPF, Karin, A-4906 Eberschwang (AT); SCHUSTER, Christian, A-4840 Vöcklabruck (AT); KRONER, Gert, A-4860 Lenzing (AT)
(74) Representative: Hanemann, Otto
(86) International application number: PCT/AT2010/000142
(87) International publication number: WO 2010/144925

(56) References cited:
- EP-A1- 1 471 169
- WO-A1-98/03708
- WO-A1-2004/081267
- JP-A- 6 057 522
- JP-A- 7 197 309
- US-A- 5 770 110
- "Terminology of man-made fibres", 1 January 2006 (2006-01-01), BISFA - International Bureau for the Standardisation of Man-Made Fibres * page 27 * * page 38 *
- Bauer, Robert: "Chemiefaser-Lexikon", 1 January 1983 (1983-01-01), Deutscher Fachverlag GmbH, Frankfurt am Main ISBN: 3 87150 185 9 * page 66 *

## Description

The present invention relates to UV protective fabrics, whereupon these fabrics are made of UV protective high-tenacity man-made cellulosic fibres. Besides the permanent and inherent protection against UV rays of the named fibre materials and thus fabrics, UV protection is still guaranteed, when the fabrics are wet and stretched. As a result of fibre swelling, the fabric construction becomes denser and as a direct result, UV transmission is significantly reduced compared to the dry and stretched state.

### Background of the Invention

Awareness of the effects and consequences of excessive exposure to UV radiation have led to an increased research interest concerning protection against UV rays. UV exposure, especially to UVA (380-315 nm) and UVB (315-280 nm) radiation, is known to cause damage of the skin like sunburn, skin-aging, allergies and even skin cancer. Dermatologists warn that particularly children should be protected from long periods of incident solar radiation, e.g. with sun protective textiles. Also for sportsmen and people, who occupationally have to remain outdoors, sun protection is vital.

In comparison to sun cream, textile materials allow for permanent protection from UV rays. However, it is hardly possible to quantify the UV shielding of textile materials by close evaluation. Well-defined standard methods, based on the determination of the Ultraviolet Protection Factor (UPF) are used in order to classify textiles according to their UV protection ability. The named standards include UV Standard 801, AS/NZS 4399:1996 and EN 13758-1. Generally speaking, sun-protective clothing must exhibit UPF values of 15 (good) to 50+ (excellent) in order to provide satisfying sun protection properties. This means that sun protective clothing has to exhibit a minimum UPF of 15 in order to be classified as sun protective. For the purposes of the present invention the AS/NZS 4399:1996 Sun Protective Clothing Evaluation and Classification Standard is used as the standard.

The UPF of fabrics varies significantly, depending on several parameters, namely fibre type, colour of the fibre und thus yarn material, constructional parameters (thickness, density, weave and yarn type, mass per unit area), presence of additives (pigments, optical brightening agents) as well as mechanical parameters (elasticity), aftertreatments, washing, laundering and moisture content. However, fabric porosity is known to be the parameter that influences UV protection most, as it determines UV transmission. Therefore, this is the key point to focus on when developing light-weight summer fabrics for beach or sports wear.

In general, high-weight, dark-coloured and thick fabrics absorb a higher amount of UV rays than light-weight, light-coloured and thin fabrics. This fact represents a severe limitation regarding the manufacture of summer clothing, since summer garments are, per definition, represented by light-weight constructions. But the most intense UV radiation is observed in summer season. So the potential of skin damage (sun burn, skin cancer), in what ever form, therefore is the highest in summer. The objective regarding UV protection, especially for beach and sports wear and even for light-weight summer work wear therefore has to be the creation of light-weight, light-coloured fabrics, which are comfortable to wear in hot season and additionally offer an optimum UV shielding ability under almost all occurring wear conditions.

Determination of the UPF of an unstretched, dry fabric sample can lead to significant misinterpretation regarding its UV protection properties, as the UPF is known to decrease under wearing conditions as a result of stretching and wetting. While stretching occurs due to the various movements of the wearer during activities, wetting may occur either by contact with water during swimming, sailing, surfing, fishing or other water sports but also simply by sweating during hiking, running, cycling, climbing, all other outdoor sports like tennis, beach volleyball etc. or even working. For example a commonly used sports wear fabric, e. g. for T-shirts, is a 170g/m² single jersey, made of 100% undyed, i. e. white cotton. In the dry state, this fabric shows a UPF of 11, measured according to AS/NZS 4399:1996. If it is stretched in the dry state according to UV Standard 801 the UPF reduces to 5.

Generally, known fabrics offer significantly lower protection from UV radiation when wet due to higher transparency. The drop in levels of protection depends on the type of fibre/fabric and the amount of moisture it absorbs. E. g. the UPF of the cotton fabric described above is 7 if wetted and stretched according to UV Standard 801. The slight increase of the UPF in the stretched state after wetting may be the effect of a swelling of the fibre.

There are several other approaches to create UV-blocking textile materials besides variation of typical construction parameters. One possible way is to treat fibres or fabrics with a UV-blocking finish, which usually contains e.g. organic UV-blocking substances or inorganic particles. But such finishes are known to lack durability. They will be removed at least partly from the fabrics during use and washing due to abrasion, leaching and the like, resulting in a loss of their UV-blocking properties.

A method commonly known in the polymer industry to overcome this disadvantage is the incorporation of functional substances into the moulded bodies during the moulding process by adding the substances to the mass before moulding, e. g. into the polymer melt or solution. Of course this method cannot be applied to the naturally grown cotton fibre.

It is known for polyester fibres to enhance the UV-blocking properties durably by incorporation of pigments during the spinning process which possess the ability to reduce transmission over the whole UV range. The utilized pigments can be of organic or inorganic origin. Since organic pigments are known to negatively affect the physical properties of the fibres to a higher extent than their inorganic counterparts, inorganic pigments such as titanium dioxide or zinc oxide, are more frequently used to affect the UV absorption and reflection properties of fibre materials. In comparison to the cotton fabric described above a fabric showing the same construction (170g/m² single jersey) but consisting of 100 % UV-blocking polyester fibres shows a nearly doubled UPF value of 20 in the dry, unstretched state. But after stretching in the dry state the UPF decreases to 8. A slight increase in UPF up to 12 can be recognized if the fabric is stretched in the wet state. As polyester does not swell with water, the water will be only adsorbed on the fibre surface and the slightly increased UPF therefore may be caused by reflection of the UV or similar effects. But in summary even such a fabric will not fulfill the requirements of a UPF of at least 15 under realistic wear conditions. Additionally fabrics made of synthetic fibres like polyester or nylon provide a very low wear comfort and bad body climate due to their low moisture absorption ability.

The incorporation of particles into man-made cellulosic fibres is already known. For example DE 195 42 533 discloses the incorporation of ceramic particles into Lyocell for the manufacture of sensor fibres. No certain compositions for these particles are mentioned. WO 2003/024891 discloses the incorporation of high amounts of TiO₂ into Lyocell for the manufacture of precursors for ceramic fibres but these precursors have completely different properties than fibres for the use in light-weight textiles. WO 96/27638 discloses the use of a masterbatch containing up to 50 % (w/w) TiO₂ in a Lyocell process for fibres for several applications, but is completely silent about the particle size and distribution of the particles as well as of the particle content in the final fibres required for light-weight UV-protective fabrics.

In view of this state of the art it is an object of this invention to provide an improved UV protection fabric, particularly for textile use as beach or sports wear or summer work wear which shows an improved UPF sufficient to protect the wearer under realistic wear conditions, as well as a good wear comfort and body climate and a tear strength sufficient to resist the rough conditions which normally occur during outdoor sports activities as well as during working.

In particular it is an object of this invention to provide an improved, durable UV protection fabric, which remains its UV shielding ability when wet and being in stretched state so that it can be used as beach wear, sports wear and even outdoor work wear for summer or other warm conditions.

### Summary of the Invention

The solution to this problem is a UV-protective fabric, containing 50 % or more of high-tenacity man-made cellulosic fibres which contain between 0,1 and 1,5 % (w/w) of an incorporated nano-scale TiO₂ pigment with a particle distribution characterized by an x₅₀ lower than 1000 nm and x₉₉ lower than 2000 nm, wherein the high-tenacity man-made cellulosic fibres are Lyocell fibres with a tenacity at break of at least 30 cN/tex in the conditioned state and at least 18 cN/tex in the wet state, both parameters evaluated according to BISFA and the fabric has a mass per unit area of 120 to 270 g/m².. Incorporated pigments shall be pigments which are added to the cellulose solution prior to spinning. Such incorporation regularly results in a very even distribution of the pigments in the fibres. This can be evaluated easily, for example by simple light microscopy of the cross-section of the fibres.

Fibres in the context of the present invention are mainly staple fibres. But also fabrics containing endless filaments will be within the scope of the invention as long as the relevant properties as outlined below are met, because filaments will generally show the same behaviour in terms of effect of the pigment, the swelling, the moisture management, mechanical strength etc.

High-tenacity man-made cellulosic fibres according to the present invention shall be man-made cellulosic fibres with a tenacity at break of at least 30 cN/tex in the conditioned state and at least 18 cN/tex in the wet state, both parameters evaluated according to BISFA.

In this fabric the cellulosic fibres contain between 0,1 and 1,5 % (w/w) of an incorporated nano-scale TiO₂ pigment with a particle distribution characterized by an x₅₀ lower than 1000 nm and x₉₉ lower than 2000 nm.

The pigment is TiO₂ as it is commercially available in sufficient quantities and quality. All particle distribution values described in the context of the present invention were measured with a HELOS/BF particle size analyser with laser diffraction and installed software.

In a particular embodiment of the invention the fabric additionally contains at least one type of synthetic fibre and/or natural cellulose fibre. The synthetic fibre can be made of polyester, polyamide, polyimide, aramide or any other suitable synthetic material and may have any denier suitable for the fabric types mentioned herein. One special type of synthetic fibre to be mentioned here additionally is Elastan which is often mixed with other fibres for the use in beach wear, sports wear and the like. The natural cellulose fibre will be mainly cotton, but can also be any other natural cellulose fibre like linen or hemp. The blending of different fibre types is common in the textile industry for different reasons. But for the objects of the present invention there are certain requirements to be achieved: E. g. blends of the high-tenacity man-made cellulosic fibres containing incorporated inorganic nano-scale pigments with polyester result in light-weight constructions with high fabric strength at an economic price. The amount of polyester present in the fabric also can be used to regulate the moisture uptake of the fabric, which may be different for different applications. Blends of the high-tenacity man-made cellulosic fibres containing incorporated inorganic nano-scale pigments with cotton fibres will result in economic fabrics with high wear comfort. Such blends can be made by mixing the fibres before making the yarn or they can be made by mixing pure yarns in warp and weft. For example a blend of 50 % of the cellulosic fibres according to the invention with 50 % of Coolmax® polyester fibre can be used for many applications in the field of beach wear and sports wear.

By incorporating UV-protective particles into the cellulosic fibres the strength of the fibres is decreased significantly. Therefore special manufacturing processes have to be used to obtain fibres with the required mechanical properties.

The fabric of the invention therefore is a fabric, wherein the high-tenacity man-made cellulosic fibres are Lyocell fibres. Lyocell fibres according to the BISFA definition are cellulosic fibres obtained by an organic solvent spinning process, wherein it is understood that an "organic solvent" means essentially a mixture of organic chemicals and water, and "solvent spinning" means dissolving and spinning without the formation of a derivative. Such processes are well-known from the literature of the last 20 years. These fibres not only show a remarkably high tenacity in the conditioned state, but also in the wet state despite their content of incorporated pigments. Another surprising advantage of the use of Lyocell fibres is that these fibres tend to fibrillate and that such fibrillation gives an additional increase in UPF. A woven Lyocell fabric made from fibres with incorporated inorganic nano-scale pigments which was fibrillated after the weaving showed a nearly doubled UPF compared to a similar fabric which was resin treated and defibrillated after weaving. This is an important advantage especially in comparison to fibres with a UV-protective finish, where no fibrils of UV-protective material occur.

According to the field of the invention the high-tenacity man-made cellulosic fibres in this fabric show a fineness of 0.8 to 3.3 dtex, preferably 0.9 to 1.7 dtex. Fibres with a higher fineness will not show sufficient mechanical properties due to the influence of the UV-protective particles. Fibres with a lower fineness, i. e. larger diameter, will not be suitable for the soft, light-weight fabrics. Mostly the fabrics are knitted or woven fabrics. Such fabrics have a mass per unit area of 120 to 270 g/m². Lighter fabrics will not show a sufficient UPF even when made of 100% incorporated fibres according to the invention. For heavier fabrics an acceptable UPF can be reached by standard fibres without incorporated inorganic nano-scale pigments.

Another object of the present invention is the use of 50 % or more of high-tenacity man-made cellulosic fibres containing between 0,1 and 1,5 % (w/w) of an incorporated nano-scale TiO₂ pigment with a particle distribution characterized by an x₅₀ lower than 1000 nm and x₉₉ lower than 2000 nm for the manufacture of an UV-protective fabric for light-weight beach, sports or work wear wherein the high-tenacity man-made cellulosic fibres are Lyocell fibres with a tenacity at break of at least 30 cN/tex in the conditioned state and at least 18 cN/tex in the wet state, both parameters evaluated according to BISFA and the fabric has a mass per unit area of 120 to 270 g/m².. The fibres can be used according to the descriptions as outlined above.

Yet disclosed herein is a method for improving the UV protection of light-weight beach, sports or work wear by using a fabric containing a blend of high-tenacity man-made cellulosic fibres which contain incorporated inorganic nano-scale pigments with non-pigmented fibres in a ratio according to the following general rules: The higher the mass per unit area of the fabric, the lower the TiO₂-content can be. But at a mass per unit area of more than 270 g/m² the use of fibres with 1% or more of TiO₂ will no further be reasonable. With regard to fibre blends the amount of UV- protective fibre has to be increased with decreasing mass per unit area. To maintain a high tear resistance of such a thin fabric, especially in the wet state, the UV-protective cellulosic fibre has to show a high tenacity. For fabrics with a very "open" construction the amount of UV-protective fibre has to be increased, too to keep a high UPF value.

The invention will now be illustrated by examples. These examples are not limiting the scope of the invention in any way.

### Example 1

1.3 dtex UV-protective Lyocell fibres with a staple length of 38 mm were manufactured according to the Lyocell process by incorporating 1 % (weight/weight) of TiO₂ (commercially available Kronos 2064) using a suitable dispersing agent. The TiO₂ dispersion was filtered before adding it to the Lyocell dope. In the filtered dispersion the TiO₂ showed a particle size distribution characterized by an x₅₀ of 570 nm and an x₉₉ of 1160 nm. The fibres show a tenacity (cond.) of 33,0 cN/tex and a tenacity (wet) of 25,5 cN/tex. The elongation at break (wet) was 14,5 %. In order to demonstrate the effect of wetness on the UPF of light-weight knitted fabrics when using single jersey fabrics made of these fibres, a series of blends of these fibres with cotton were ring-spun into 20tex yarns and therefrom single jersey fabrics, having a mass per unit area of 140 g/m², were fabricated. The fabrics were made wet and stretched, using a biaxial stretching frame according to UV Standard 801. Subsequently the UPF was determined according to the AS/NZS 4399:1996 Sun Protective Clothing Evaluation and Classification Standard. The obtained results are summarized in Figure 1. It can clearly be deduced that the higher the amount of UV-protective Lyocell in the fibre blend, the higher the UPF in the wet and stretched state. For fabrics, consisting of 70% (or even higher) UV-protective Lyocell, the UPF was found to be more than doubled when comparing the dry and the wet stretched samples.

### Example 2

1.3 dtex UV-protective Modal fibres with a staple length of 39 mm were manufactured according to the process described in the Austrian patent publication AT 287905 by incorporating 1 % (weight/weight) of TiO₂ (commercially available Kronos 2064) using a suitable dispersing agent. The TiO₂ dispersion was filtered before adding it to the spinning dope. In the filtered dispersion the TiO₂ showed a particle size distribution characterized by an x₅₀ of 570 nm and an x₉₉ of 1160 nm.. The fibres show a tenacity (cond.) of 34,0 cN/tex and a tenacity (wet) of 19,0 cN/tex. The elongation at break (wet) was 15,0 %. For further demonstration of how the fibre swelling positively affects UV protection, these UV-protective Modal fibres as well as the UV-protective Lyocell fibres of example 1, were ring-spun into 20tex yarns and therefrom single jersey fabrics having a mass per unit area of 170 g/m², were fabricated. Before evaluation of their UV protection ability, the fabrics were wetted and stretched according to UV Standard 801. Subsequently the UPF was determined according to the AS/NZS 4399:1996 Sun Protective Clothing Evaluation and Classification Standard. A summary of the obtained results is given in Figure 2. As expected, wetting the fabrics had a significant effect on UPF values, greatly depending on the nature of fibre. The UPF values for UV-protective Modal and UV-protective Lyocell fabrics increased in the wet state, which is in accordance with the previous findings described in Example 1. It is clearly demonstrated that UV-protective Modal or UV-protective Lyocell retain their UV protection ability also in the wet state, which is confirmed by UPF values of 20 and higher. Figure 2 also shows the less performing results for 170 g/m² single jersey fabrics made of regular cotton and of commercially available 1,3 dtex polyethylene terephthalate fibres containing 1 % (w/w) of TiO₂.

Summarising these results it can be concluded that the swelling potential of UV-protective Modal or UV-protective Lyocell fibres represents a remarkable benefit when designing UV protective clothing for beach wear, sports wear and even work wear.

## Claims

1. UV-protective fabric, containing 50 % or more of high-tenacity man-made cellulosic fibres which contain between 0,1 and 1,5 % (w/w) of an incorporated nano-scale TiO₂ pigment with a particle distribution **characterized by** an x₅₀ lower than 1000 nm and x₉₉ lower than 2000 nm, wherein the high-tenacity man-made cellulosic fibres are Lyocell fibres with a tenacity at break of at least 30 cN/tex in the conditioned state and at least 18 cN/tex in the wet state, both parameters evaluated according to BISFA and the fabric has a mass per unit area of 120 to 270 g/m².

2. Fabric according to claim 1, wherein the fabric additionally contains at least one type of synthetic and/or cellulose fibre.

3. Fabric according to claim 1, wherein the high-tenacity man-made cellulosic fibres show a fineness of 0.8 to 3.3 dtex.

4. Fabric according to claim 1, wherein the fabric is a knitted or a woven fabric.

5. Use of 50 % or more of high-tenacity man-made cellulosic fibres containing between 0,1 and 1,5 % (w/w) of an incorporated nano-scale TiO₂ pigment with a particle distribution **characterized by** an x₅₀ lower than 1000 nm and x₉₉ lower than 2000 nm for the manufacture of an UV-protective fabric for light-weight beach, sports or work wear wherein the high-tenacity man-made cellulosic fibres are Lyocell fibres with a tenacity at break of at least 30 cN/tex in the conditioned state and at least 18 cN/tex in the wet state, both parameters evaluated according to BISFA and the fabric has a mass per unit area of 120 to 270 g/m².

## Patentansprüche

1. UV-Schutz-Flächengebilde, enthaltend 50% oder mehr hochfeste Man-Made-Cellulosefasern, die zwischen 0,1 und 1,5 Gew.-% eines eingebundenen nanoskaligen TiO₂-Pigments mit einer Partikelverteilung, die durch einen x₅₀-Wert kleiner als 1000 nm und einen x₉₉-Wert kleiner als 2000 nm gekennzeichnet ist, enthalten, wobei die hochfesten Man-Made-Cellulosefasern Lyocellfasern mit einer Reißfestigkeit von mindestens 30 cN/tex im konditionierten Zustand und von mindestens 18 cN/tex im nassen Zustand sind, wobei beide Parameter gemäß BISFA evaluiert werden, und das Flächengebilde ein Flächengewicht von 120 bis 270 g/m² aufweist.

2. Flächengebilde nach Anspruch 1, wobei das Flächengebilde zusätzlich mindestens eine Art von Synthese- und/oder Cellulosefaser enthält.

3. Flächengebilde nach Anspruch 1, wobei die hochfesten Man-Made-Cellulosefasern eine Feinheit von 0,8 bis 3,3 dtex aufweisen.

4. Flächengebilde nach Anspruch 1, wobei das Flächengebilde ein Gestrick bzw. Gewirk oder ein Gewebe ist.

5. Verwendung von 50% oder mehr hochfesten Man-Made-Cellulosefasern, die zwischen 0,1 und 1,5 Gew.-% eines eingebundenen nanoskaligen TiO₂-Pigments mit einer Partikelverteilung, die durch einen x₅₀-Wert kleiner als 1000 nm und einen x₉₉-Wert kleiner als 2000 nm gekennzeichnet ist, enthalten, zur Herstellung eines UV-Schutz-Flächengebildes für leichte Strand-, Sport- oder Arbeitsbekleidung, wobei die hochfesten Man-Made-Cellulosefasern Lyocellfasern mit einer Reißfestigkeit von mindestens 30 cN/tex im konditionierten Zustand und von mindestens 18 cN/tex im nassen Zustand sind, wobei beide Parameter gemäß BISFA evaluiert werden, und das Flächengebilde ein Flächengewicht von 120 bis 270 g/m² aufweist.

## Revendications

1. Étoffe de protection anti-UV contenant 50 % ou plus de fibres de cellulose artificielles à haute résistance qui contiennent entre 0,1 et 1,5 % en masse d'un pigment de TiO₂ incorporé de l'ordre du nanomètre, avec une répartition des particules **caractérisée par** x₅₀ inférieur à 1 000 nm et x₉₉ inférieur à 2 000 nm, lesdites fibres de cellulose artificielles à haute résistance étant des fibres Lyocell d'une résistance à la rupture d'au moins 30 cN/tex à l'état conditionné, et d'au moins 18 cN/tex à l'état humide, ces deux paramètres étant évalués conformément au BISFA, et l'étoffe présentant un poids surfacique compris entre 120 et 270 g/m².

2. Étoffe selon la revendication 1, l'étoffe contenant en plus au moins un type de fibre synthétique et/ou de cellulose.

3. Étoffe selon la revendication 1, les fibres de cellulose artificielles à haute résistance présentant une finesse de 0,8 à 3,3 dtex.

4. Étoffe selon la revendication 1, l'étoffe étant un tricot ou un tissu.

5. Utilisation de 50 % ou plus de fibres de cellulose artificielles à haute résistance qui contiennent entre 0,1 et 1,5 % en masse d'un pigment de TiO₂ incorporé de l'ordre du nanomètre, avec une répartition des particules **caractérisée par** x₅₀ inférieur à 1 000 nm et x₉₉ inférieur à 2 000 nm, pour la fabrication d'une étoffe de protection anti-UV pour vêtements légers de plage, de sport et de travail, lesdites fibres de cellulose artificielles à haute résistance étant des fibres Lyocell d'une résistance à la rupture d'au moins 30 cN/tex à l'état conditionné, et d'au moins 18 cN/tex à l'état humide, ces deux paramètres étant évalués conformément au BISFA, et l'étoffe présentant un poids surfacique compris entre 120 et 270 g/m².
